

- [54] CUMULENE-RESIN BINDER  
PHOTOCONDUCTIVE ELEMENTS  
[75] Inventor: Robert G. Blanchette, Mayfield  
Heights, Ohio  
[73] Assignee: Addressograph-Multigraph  
Corporation, Cleveland, Ohio  
[22] Filed: Mar. 26, 1973  
[21] Appl. No.: 345,104

**Related U.S. Application Data**

- [60] Continuation of Ser. No. 244,993, April 17, 1972,  
abandoned, which is a division of Ser. No. 78,628,  
Oct. 6, 1970, Pat. No. 3,674,473, which is a  
continuation-in-part of Ser. No. 771,352, Oct. 28,  
1968, abandoned.  
[52] U.S. Cl. .... 96/1.6, 96/1.5  
[51] Int. Cl. .... G03g 5/06, G03g 13/22  
[58] Field of Search..... 96/1.5, 1.6

[56] **References Cited**

UNITED STATES PATENTS

- 3,556,785 1/1971 Baltazzi..... 96/1.5  
3,674,473 7/1972 Blanchette ..... 96/1.5

FOREIGN PATENTS OR APPLICATIONS

- 41-18,467 10/1966 Japan..... 96/1.5

*Primary Examiner*—Roland E. Martin, Jr.  
*Attorney, Agent, or Firm*—Sol L. Goldstein; Michael  
A. Kondzella

[57] **ABSTRACT**

A photoelectrostatic member in a process for electrostatic imaging includes a photoconductive layer containing a compound selected from the general class of cumulenes dispersed in a resin binder applied to the member. The cumulene compounds useful in the instant invention have of the following general formulas:



where X represents an alkyl, hydrogen, halogen or nitro substituent; Q<sub>1</sub> and Q<sub>2</sub> can be:



indene or fluorene;

n can be an integer from 1 through 6;

R is lower alkyl, aryl or hydrogen; R<sub>1</sub> and R<sub>2</sub> can be

aryl,

substituted aryl,

heterocyclic ring structures; and where Q<sub>1</sub>, Q<sub>2</sub>, or R<sub>1</sub> and R<sub>2</sub> can be the same or different.

**6 Claims, No Drawings**

## CUMULENE-RESIN BINDER PHOTOCONDUCTIVE ELEMENTS

## CROSS REFERENCE

This application is a continuation of application Ser. No. 244,993, filed Apr. 17, 1972, now abandoned, which is a divisional application divided out of application Ser. No. 78,628, filed Oct. 6, 1970 now issued as U.S. Pat. No. 3,674,473, which application was a continuation in part of application Ser. No. 771,352, filed Oct. 28, 1968, now abandoned.

## BACKGROUND OF THE INVENTION

This invention relates to organic photoconductive materials and, more particularly, to a class of compounds known as cumulenes which contain a unit of " $m$ " carbon atoms with  $(m-1)$  double bonds between them, where  $m$  is an integer equal to or greater than 3.

Photoelectrostatic imaging processes involve the use of a photoconductive medium which is charged in the dark, exposed to a pattern of light and shadow thereby producing a charge pattern corresponding to the image portions of the original design to be reproduced. This charge pattern is then developed by applying an electrostatically attractive powder generally known as toner in this art.

The photoconductive medium usually comprises a conductive support to which has been applied a photoconductive layer or film in which the active photoconductive material is selenium, zinc oxide, or an organic compound. A wide variety of organic photoconductive materials are known and have been suggested, some of which are polymeric in nature and in themselves form a uniform continuous photoconductive film. Other types of organic photoconductive compounds can be used which are crystalline and therefore lend themselves to being dispersed through organic resin binders and applied to a conductive support.

## SUMMARY OF THE INVENTION

In accordance with the present invention a new class of organic photoconductors is provided having any one of the following general formulas:

## List of compounds formula

|        |                                                                                     | Name                       |
|--------|-------------------------------------------------------------------------------------|----------------------------|
| 1..... |  | Bifluorenylidene-ethylene. |
| 2..... |  | Tetraphenyl-hexapentaene.  |
| 3..... |  | Tetraphenyl-butatriene.    |



where  $X$  represents an alkyl, hydrogen, halogen or nitro substituent;  $Q_1$  and  $Q_2$  can be:



indene, or fluorene;

15  $n$  can be an integer from 1 through 6;  $R$  is a lower alkyl, aryl or hydrogen;  $R_1$  and  $R_2$  can be aryl, substituted aryl, heterocyclic ring structures, fused arenic ring structures; and  $Q_1$ ,  $Q_2$ , or  $R_1$  and  $R_2$  can be the same or different, said compound being dispersed in a resin binder.

The support on which the photoconductive material is applied may be paper which has been treated to render it conductive or it can be metal or metal foil such as aluminum, copper, or zinc. Generally, it is understood in this art that the base support must have a conductivity in the range from  $10^{-11}$  mhos per centimeter to the conductivity of metal.

It is the general object of the present invention to provide an improved organic photoconductive medium formulated with compounds which contain a unit of  $(m)$  carbon atoms with  $(m-1)$  double bonds between them where  $(m)$  is an integer equal to or greater than 3.

35 It is another object of this invention to provide a photoconductive material comprised of organic crystalline materials selected from the general class of cumulenes.

It is still another object of this invention to provide a photoconductive member formulated with an organic crystalline material dispersed in an insulating resin binder which formulation is simple to prepare and which photoconductive member gives an increased photo response.

## DESCRIPTION OF THE INVENTION:

Compounds which are typical of the cumulene-type materials useful in the preparation of the photoconductive members of this invention are the following:

-Continued

## List of compounds formula

## Name

|         |                                                                                     |                                                               |
|---------|-------------------------------------------------------------------------------------|---------------------------------------------------------------|
| 4.....  |    | Tetra-(m-bromophenyl) hexapentaene.                           |
| 5.....  |    | Bis(3,6-dinitrofluorenylidene)ethylene.                       |
| 6.....  |    | 1,4-bis(1,1-diphenyl-4-ethyl-4-butatrienyl)benzene.           |
| 7.....  |    | 1,4-diphenyl-1,4-di-2-thienylbuta- triene.                    |
| 8.....  |   | 1-(inden-1-ylidene)-3-diphenyl- propadiene.                   |
| 9.....  |  | 1,4-bis(1,1-di-4-bromophenyl-4- phenyl-4-butatrienyl)benzene. |
| 10..... |  | 1,4-bis(1,1-diphenylbutatrienyl)-2- nitrobenzene.             |
| 11..... |  | Tetraphenylpentatetraene.                                     |
| 12..... |  | 1,4-di(3-methylphenyl)-1,4- diphenylbutatriene.               |
| 13..... |  | 1,4-diphenyl-1,4-di(4-phenyl- phenyl)butatriene.              |

## List of compounds formula

## Name

|         |  |                                                         |
|---------|--|---------------------------------------------------------|
| 14..... |  | 1,4-di(2-naphthyl)-1,4-diphenylbutatriene.              |
| 15..... |  | 1,4-di(2,4-dimethylphenyl)-1,4-diphenylbutatriene.      |
| 16..... |  | 1,4-di(2,5-dimethylphenyl)-1,4-diphenylbutatriene.      |
| 17..... |  | 1,4-di(3,4-dimethylphenyl)-1,4-diphenylbutatriene.      |
| 18..... |  | 1,4-di(2-methylphenyl)-1,4-diphenylbutatriene.          |
| 19..... |  | 1,4-di(4-fluorophenyl)-1,4-diphenylbutatriene.          |
| 20..... |  | 1,4-diphenyl-1,4-di(3-phenylphenyl)butatriene.          |
| 21..... |  | 1,4-diphenyl-1,4-di(3-trifluoromethylphenyl)butatriene. |
| 22..... |  | 1,4-diphenyl-1,4-di-p-terphenylbutatriene.              |

The photoconductive crystalline materials of this invention can be prepared by a number of well-known methods as described in the following references: Chapter 13, "Cumulenes", by H. Fisher, "The Chemistry of Alkenes," S. Patai, ed., Interscience Publishers, London, New York, Sydney, 1,964, page 1025; 65 "Cumulenes," Cadiot, Chodkiewicz, and Rauss Godineau, Bulletin of the Chemical Society of France, 2126, (1961).

60 The preparation of the cumulenes of this invention such as, for example, 1,1,4,4-tetraphenylbutatriene, may be accomplished by the reduction of the appropriately substituted 1,1,4,4-tetraphenylbutynediol obtained from the reaction of a benzophenone and acetylene, with potassium iodide and sulphuric acid. The symmetrically substituted hexapentaenes may be obtained by potassium hydroxide-acetic acid anhydride condensation of 1,1-diphenylpropargyl alcohol. The

compound 1,2-bifluorenylideneethylene may be obtained by the treatment of 9-bromoethylenefluorene with potassium amide in liquid ammonia as described by Hauser and Lednicer, Journal of Organic Chemistry, 22, page 1,248 (1957).

Photoelectrostatic members of this invention may be prepared by mixing the particulate crystalline material in a suitable solvent such as chlorobenzene, toluene, methylene chloride, or tetrahydrofuran with a suitable resin. The mixture is then ball milled for sufficient time until complete uniform blending of all the ingredients is accomplished. This usually requires anywhere from 15 - 24 hours. Such film forming resins as polyvinyl acetate, polyvinyl ethers, polystyrene, alkyd resins, phenylformaldehyde resins, styrene-butadiene copolymers, and polyamide resins may be employed as binders. The resin binder may comprise from 10 percent - 75 percent by weight of the total weight of solids present in the photoconductive layer.

After the mixture is ball milled it is applied to a suitably conductive substrate by conventional coating techniques such as a meniscus coater, a wire wound rod or doctor blade at the rate of 0.5 grams to 2.0 grams per square foot, preferably 0.5 to 1 gram per square foot to produce a film thickness in the range of 0.1 mil to 5.0 mils in thickness, preferably in the range of 0.2 to 0.5 mil thickness. Evaporation of the solvent may be carried out by passing the coated web material through a forced air oven-type dryer.

It is generally known in the art dealing with the preparation of photoconductive members, whether they are of the inorganic or organic type, that the photoresponse of such members may be improved through the addition of certain sensitizers or additives. In the case of inorganic photoconductive materials such as zinc oxide, these additives are in the form of dyes which increase the photoresponse by the mechanism of extending the spectral response of the photoconductive member. In the case of organic photoconductors involving donor-acceptor type materials or charge transfer type systems, the use of additives tends to extend the spectral response range or shift the spectral sensitivity into the visible portion of the spectrum and also tends to increase the sensitivity in a given spectral sensitivity range and thereby achieving a more efficient system.

It should be pointed out that the photoconductive materials of the instant invention exhibit the property of photoconductivity independent of the use of such additives or in fact independently of resin binders with which they may be combined. Such photoconductivity is determined by measuring the photocurrent of the materials coated on nesa glass surface cells or electrodes. The current which results, results when the charged nesa glass surface cell, which is coated with the specific chemical compound in a suitable solvent and evaporated to dryness, is illuminated with electromagnetic radiation represents the photocurrent. When referring to nesa glass surface cell measurement, the photoresponse is indicated in terms of the ratio of the photocurrent which results upon illumination of electromagnetic radiation to the dark current values.

Photoresponse of the compounds of the instant invention respond to radiation in the range of 375 to 600 millimicrons. While the compounds may be used to advantage without the use of sensitizers in this range of sensitivity to electromagnetic radiation, it is desirable to increase the degree of photoresponse and/or extend

the range of the spectral response. The organic photoconductors of the instant invention when measured on a nesa glass surface cell, exhibit a ratio of photocurrent to dark current in the range of 30 to 1,000.

5 The cumulenes as a class of photoconductors exhibit an increase in photoresponse upon the addition of certain additives which are chemical sensitizers such as pi-type acids such as disclosed in copending application Ser. No. 679,246 and Ser. No. 707,413, filed in the name of Evan S. Baltazzi, which inventions are assigned to the same assignee as the instant invention.

The following list of pi-type sensitizers is representative of compounds of the dicyanomethylene fluorene type and the butenolides.

- 9-(dicyanomethylene)-3-nitrofluorene
- 9-(dicyanomethylene)-2,4-dinitrofluorene
- 9-(dicyanomethylene)-2,4,7-trinitrofluorene
- 9-(dicyanomethylene)-2,5-dinitrofluorene
- 9-(dicyanomethylene)-2,6-dinitrofluorene
- 9-(dicyanomethylene)-2,7-dinitrofluorene
- 9-(dicyanomethylene)-2,4,5,7-tetranitrofluorene
- 9-(dicyanomethylene)-3,6-dinitrofluorene
- 9-(dicyanomethylene)-2,4-dicyanofluorene
- 9-(dicyanomethylene)-2,4,7-tricyanofluorene
- 9-(dicyanomethylene)-2,4,5,7-tetracyanofluorene
- 9-(dicyanomethylene)-2,4-difluoromethylfluorene
- 9-(dicyanomethylene)-2,4,7-trifluoromethylfluorene
- 9-(dicyanomethylene)-2,4,5,7-tetr trifluoromethylfluorene
- 9-(dicyanomethylene)-2,4,5,7-tetr trifluoromethylfluorene
- 9-(dicyanomethylene)-2,4-dimethylfluorene
- 9-(dicyanomethylene)-2,4,7-trimethylfluorene
- 9-(dicyanomethylene)-2,4,5,7-tetramethylfluorene
- 9-(dicyanomethylene)-2,4-dibutoxyfluorene
- 9-(dicyanomethylene)-2,4,7-tributoxyfluorene
- 9-(dicyanomethylene)-2,4,5,7-tetrabutoxyfluorene
- 9-(dicyanomethylene)-2,4-dichlorofluorene
- 9-(dicyanomethylene)-2,4,7-trichlorofluorene
- 9-(dicyanomethylene)-2,4,5,7-tetrachlorofluorene
- 2-Phenyl-4 (9-fluorenylidene)-5-oxazolone
- 2-Phenyl-4 (2,4-Dinitro-9-fluorenylidene)-5-oxazolone
- 2-Phenyl-4 (2,4,7-Trinitro-9-fluorenylidene)-5-oxazolone
- 2-Phenyl-4 (2,5-Dinitro-9-fluorenylidene)-5-oxazolone
- 2-Phenyl-4 (2,6-Dinitro-9-fluorenylidene)-5-oxazolone
- 2-Phenyl-4 (2,7-Dinitro-9-fluorenylidene)-5-oxazolone
- 2-Phenyl-4 (2,4,5,7-Tetranitro-9-fluorenylidene)-5-oxazolone
- 2-Phenyl-4 (3,6-Dinitro-9-fluorenylidene)-5-oxazolone
- 2-Phenyl-4 (2,4-Dicyano-9-fluorenylidene)-5-oxazolone
- 2-Phenyl-4 (2,4,7-tricyano-9-fluorenylidene)-5-oxazolone
- 2-Phenyl-4 (2,4,5,7-Tetracyano-9-fluorenylidene)-5-oxazolone
- 2-Phenyl-4 (2,4-di-trifluoromethyl-9-fluorenylidene)-5-oxazolone
- 2-Phenyl-4 (2,4-Dichloro-9-fluorenylidene)-5-oxazolone
- 2-Phenyl-4 (2,4,7-Trichloro-9-fluorenylidene)-5-oxazolone
- 2-Phenyl-4 (2,4,5,7-Tetrachloro-9-fluorenylidene)-5-oxazolone

$\alpha$ -(9-fluorenylidene)- $\gamma$ -phenyl- $\Delta^B$ , $\gamma$ -butenolide  
 $\alpha$ -(2,4-Dinitro-9-fluorenylidene)- $\gamma$ -phenyl- $\Delta^B$ , $\gamma$ -butenolide  
 $\alpha$ -(2,4,7-Trinitro-9-fluorenylidene)- $\gamma$ -phenyl- $\Delta^B$ , $\gamma$ -butenolide  
 $\alpha$ -(2,5-Dinitro-9-fluorenylidene)- $\gamma$ -phenyl- $\Delta^B$ , $\gamma$ -butenolide  
 $\alpha$ -(2,6-Dinitro-9-fluorenylidene)- $\gamma$ -phenyl- $\Delta^B$ , $\gamma$ -butenolide  
 $\alpha$ -(2,7-Dinitro-9-fluorenylidene)- $\gamma$ -phenyl- $\Delta^B$ , $\gamma$ -butenolide  
 $\alpha$ -(2,4,5,7-Tetranitro-9-fluorenylidene)- $\gamma$ -phenyl- $\Delta^B$ , $\gamma$ -butenolide  
 $\alpha$ -(3,6-Dinitro-9-fluorenylidene)- $\gamma$ -phenyl- $\Delta^B$ , $\gamma$ -butenolide  
 $\alpha$ -(2,4-Dicyano-9-fluorenylidene)- $\gamma$ -phenyl- $\Delta^B$ , $\gamma$ -butenolide  
 $\alpha$ -(2,4,7-Tricyano-9-fluorenylidene)- $\gamma$ -phenyl- $\Delta^B$ , $\gamma$ -butenolide  
 $\alpha$ -(2,4,5,7-Tetracyano-9-fluorenylidene)- $\gamma$ -phenyl- $\Delta^B$ , $\gamma$ -butenolide  
 $\alpha$ -(2,4-Difluoromethyl-9-fluorenylidene)- $\gamma$ -phenyl- $\Delta^B$ , $\gamma$ -butenolide  
 $\alpha$ -(2,4-Dichloro-9-fluorenylidene)- $\gamma$ -phenyl- $\Delta^B$ , $\gamma$ -butenolide  
 $\alpha$ -(2,4,7-Trichloro-9-fluorenylidene)- $\gamma$ -phenyl- $\Delta^B$ , $\gamma$ -butenolide  
 $\alpha$ -(2,4,5,7-Tetrachloro-9-fluorenylidene)- $\gamma$ -phenyl- $\Delta^B$ , $\gamma$ -butenolide

In addition to the sensitizers referred to above, a large number of substances are disclosed in U.S. Pat. No. 3,037,861, issued to Helmut Hoegl, et al, dated June 5, 1962, which discloses compounds from the class of mineral acids, organic sulfonic acids, organic phosphonic acids, nitrophenols, acid anhydrides, metal halides of the metals and metalloids of the groups 1 B - 2 through group 8 of the periodic system, boron halide compounds, organic substances containing CO-groups which are substantially monomeric, aldehydic compounds and ketonic materials.

The mechanism by which these additives enhance or increase the photoresponse is not fully understood. Reference to increase in photoresponse of the photoconductive materials when applied in a uniform film to a paper substrate may be defined in terms of the rate of voltage drop  $dv/dt$  as a function of voltage. It is this measured rate of voltage drop, which when compared to photoconductive members without sensitizers, is increased over the same range of electromagnetic radiation which can vary from 360 millimicrons to 700 millimicrons.

The photosensitivity of the members of the instant invention may be defined in terms of a conventional zinc oxide resin binder photoconductive member. The photosensitivity of the latter for the purpose of this invention has generally been assigned the arbitrary numerical rating of 150 units representing the standard or normal photoresponse when such exposure is accomplished using a tungsten-type filament source.

The sensitivity of the members of this invention which did not include the pi-type acids received a rating of 1.0 relative to the standard zinc oxide member.

The photoelectrostatic members to which had been added the pi-type acids and which were exposed to a tungsten filament type lamp received a photosensitivity rating in the range of 80 to 210 units on this scale of

comparison. In all cases the developed images which are obtained using the instant photoconductive members are of high contrast and good image density.

The amount of sensitizer employed may range from 0.1 to 5.0 moles per hundred moles of organic photoconductor. The preferred amount of sensitizer is between 0.5 to 1.5 moles per hundred moles of organic photoconductor. A typical sensitizer that may be used is 9-(dicyanomethylene)-2,4,7-trinitrofluorene.

The process of making a reproduction utilizing the photoelectrostatic members of this invention involves applying a sensitizing electrostatic charge to the photoconductive layer in the range of 200 to 1,000 volts by means of a corona discharge electrode which is connected to a high potential source of from 4,000 to 7,000 volts. The materials of this invention may be charged either positively or negatively but exhibit a marked increase in sensitivity when charged positively. The charged layer upon receiving electrostatic charge in the dark, becomes sensitive to electromagnetic radiation and is then exposed to a pattern of light and shadow by directing the radiation through a light transmitting original which is placed in contact over the photoconductive layer or by illuminating a graphic original with suitable electromagnetic radiation and then projecting the reflected pattern of light and shadow through a lens system onto the photoelectrostatic member.

Exposing the photoconductive layer to a pattern of light and shadow produces a corresponding electrostatic image with the charged area corresponding to the shadow portions and in the light struck areas the charge is dissipated. The charged pattern or image is rendered visible by the application of a suitable toner which adheres to the image portions. Positively oriented toners are generally employed where the sensitizing charge is negative and reversal oriented toners are used for positively charged members, both systems producing a positive print from a positive original. The make-up of these toners is generally well known in the art and need not be further described here.

The material image is then fixed directly on the member or it may be transferred under controlled conditions to a receiving sheet, such as plain paper, and then fixed. The material image may be fixed by exposing the toner to a source of heat which causes the material to coalesce and fuse to support. In the circumstance that the toners are pressure responsive, they can be fixed by the application of pressure such as passing the members between the set of pressure rollers.

The following examples are presented for illustrating the present invention without limiting the scope thereof.

#### EXAMPLE I

A photoelectrostatic member was prepared by mixing 10 grams of bifluorenylidene ethylene and 10 grams of styrenebutadiene copolymer sold by Goodyear Tire and Rubber Company under the tradename "Pliolite S5D" in 80 grams of toluene. The mixture was ball milled at room temperature until complete blending was achieved requiring approximately 18 to 24 hours. The mix was then applied to a suitable conductive support material such as aluminized mylar — 5 mil thickness using conventional coating equipment such as a meniscus coater or a wire wound rod. The solution was applied at a rate sufficient to produce a photoconduc-

tive layer of about 0.2 to 0.3 mil in thickness after the evaporation of the solvent. The coating weight was 0.5 grams per square foot. Evaporation of the toluene from the solution is accomplished by passing the coated web through forced hot air ovens maintained between 90° C. to 135° C.

The resulting member was charged positively and exposed to a pattern of light and shadow producing a latent electrostatic image thereon which was then developed by the application of a suitable electroscopic powder or toner. The photoresponse of the photoelectrostatic member was rated about 1.0 since the electro-photographic member was not sensitized.

I claim:

1. An electrostatic imaging process for making reproductions of a graphic original on a photoelectrostatic member comprising the steps of applying a blanket of electrostatic charge to the surface of said member, exposing said charged surface to a pattern of light and shadow, producing a latent electrostatic image thereon, and developing said latent electrostatic image by the application of toner powder thereon, said photoelectrostatic member comprising a conductive base support having a photoconductive layer applied thereon comprising an organic photoconductive compound dispersed in a resin binder, said photoconductive compound having one of the following formulas:



5

where x is alkyl, halogen, hydrogen or nitro, n is an integer from 1 through 6; Q<sub>1</sub> and Q<sub>2</sub> are selected from the group consisting of:



10

indene, or fluorene;

R is selected from the group consisting of lower alkyl, aryl or hydrogen; R<sub>1</sub> and R<sub>2</sub> can be aryl, substituted aryl or thiaryl; and wherein Q<sub>1</sub> and Q<sub>2</sub> or R<sub>1</sub> and R<sub>2</sub> can be the same or different.

2. The process as claimed in claim 1 in which said photoelectrostatic member contains a pi-type sensitizer.

3. The process as claimed in claim 1 in which said photoelectrostatic member contains a sensitizer selected from the group consisting of dicyanomethylene fluorenes, phenyl fluorenylidene oxazolones and  $\gamma$ -phenyl- $\Delta\beta\gamma$ -butenolides.

4. The process as claimed in claim 1 in which said sensitizer is present in the amount of from about 0.1 to about 5.0 mole percent, based on said organic photoconductive compound.

5. The process as claimed in claim 1 in which said sensitizer is from about 0.25 to about 2.5 mole percent, based on said organic photoconductive compound, of 9-dicyanomethylene-2, 4, 7-trinitrofluorene.

6. The process as claimed in claim 1 in which said sensitizer is from about 0.5 to about 5.0 mole percent, based on said organic photoconductive compound, of 2-phenyl-4-(2, 4, 5, 7-tetranitro-9-fluorenylidene)-5-oxazolone.

\* \* \* \* \*

45

50

55

60

65

UNITED STATES PATENT OFFICE Page 1 of 2  
CERTIFICATE OF CORRECTION

Patent No. 3,841,871 Dated October 15, 1974

Inventor(s) Robert G. Blanchette

It is certified that error appears in the above-identified patent and that said Letters Patent are hereby corrected as shown below:

ABSTRACT: Insert the following formula after the sentence "The cumulene compounds useful in the instant invention have of the following general formulas:"



Col. 4, line 1, change "Tetra-(m-bromophenyl hexapentaene" to --  
Tetra-(m-bromophenyl) hexapentaene --

Col. 5, Formula 21, This formula should read as follows:



Col. 9, line 4, should read as follows:  $\alpha$ -(2,4,7-Trinitro-9-fluorenylidene)-  
 $\gamma$ -phenyl-  $\Delta^8$ ,  $\gamma$ -

Col. 9, line 8, should read as follows:  $\alpha$ -(2,6-Dinitro-9-fluorenylidene)-  
 $\gamma$ -phenyl-  $\Delta^8$ ,  $\gamma$ -

UNITED STATES PATENT OFFICE Page 2 of 2  
CERTIFICATE OF CORRECTION

Patent No. 3,841,871

Dated October 15, 1974

Inventor(s) Robert G. Blanchette

It is certified that error appears in the above-identified patent and that said Letters Patent are hereby corrected as shown below:

ol. 11, lines 28 - 35, delete the formulas in brackets.

ol. 11, lines 36 - 41, This formula should read as follows:



ol. 12, line 14, change "can be" to -- are selected from the group consisting of --.

ol. 12, line 34, should read as follows: 9-(dicyanomethylene)-2,4,7-trinitrofluorene.

ol. 12, line 37, change "1" to -- 2 --.

Signed and Sealed this  
eighteenth Day of May 1976

[SEAL]

Attest:

RUTH C. MASON  
Attesting Officer

C. MARSHALL DANN  
Commissioner of Patents and Trademarks